# EUROPEAN PATENT APPLICATION

(11) **EP 4 707 930 A1**
(43) Date of publication of application: **11.03.2026**
(21) Application number: 25157005.7
(22) Date of filing: 11.02.2025
(51) Int. Cl.: G03G 5/05

(54) **ELECTROPHOTOGRAPHIC PHOTORECEPTOR, PROCESS CARTRIDGE, AND IMAGE FORMING APPARATUS**

(30) Priority: 04.09.2024 JP 2024152719
(71) Applicant: FUJIFILM Business Innovation Corp., Minato-ku Tokyo (JP)
(72) Inventor: KANEKO, Ryota, Ebina-shi, Kanagawa (JP)
(74) Representative: Kurig, Thomas

(57) **Abstract**

An electrophotographic photoreceptor includes a conductive substrate, a charge generation layer that is disposed on the conductive substrate, and a charge transport layer that is disposed on the charge generation layer and contains a binder resin, a charge transport material, and metal oxide particles, in which, in a case where a cross section of the charge transport layer is observed, a proportion of single particles of the metal oxide particles to a total of the single particles and aggregated particles of the metal oxide particles is 60% by number or more.

## Description

### BACKGROUND OF THE INVENTION

### (i) Field of the Invention

The present invention relates an electrophotographic photoreceptor, a process cartridge, and an image forming apparatus.

### (ii) Description of Related Art

JP2023-054576A discloses "electrophotographic photoreceptor that includes at least a lamination-type photosensitive layer in which a charge generation layer containing a charge generation substance and a charge transport layer containing a charge transport substance are laminated in this order on a conductive support, or includes at least the lamination-type photosensitive layer and a surface protective layer laminated thereon, in which both or either one of the charge transport layer and the surface protective layer contains a light absorber, an outermost surface layer of the electrophotographic photoreceptor contains a silica filler, the outermost surface layer has a transmittance of 50% or more with respect to light having a wavelength of 600 nm, and a ratio T600/T550 of a transmittance T600 with respect to light having a wavelength of 600 nm to a transmittance T550 with respect to light having a wavelength of 550 nm is 1.10 or more and 2.20 or less".

JP2023-069379A discloses "electrophotographic photoreceptor that includes a conductive support and a photosensitive layer formed on the conductive support, in which the photosensitive layer is composed of one or more layers, a surface layer of the photosensitive layer contains a binder resin, silica particles, and a charge transport substance, a ten-point average roughness Rz of a surface of the surface layer is 0.08 µm or more and 0.80 µm or less, an average interval Sm of unevenness on the surface of the surface layer is more than 15 µm and 120 µm or less, and a ratio Sm/Rz of the average interval Sm to the ten-point average roughness Rz is 30 or more and 500 or less".

### SUMMARY OF THE INVENTION

An object of the present invention is to provide an electrophotographic photoreceptor including a conductive substrate, a charge generation layer that is disposed on the conductive substrate, and a charge transport layer that is disposed on the charge generation layer and contains a binder resin, a charge transport material, and metal oxide particles, in which the electrophotographic photoreceptor has excellent abrasion resistance and electrical properties, as compared with a case where, when a cross section of the charge transport layer is observed, a proportion of single particles of the metal oxide particles to a total of the single particles and aggregated particles of the metal oxide particles is less than 60% by number.

Methods for achieving the above object include the following aspects.
<1> According to a first aspect of the present invention, there is provided an electrophotographic photoreceptor including:
   a conductive substrate;
   a charge generation layer that is disposed on the conductive substrate; and
   a charge transport layer that is disposed on the charge generation layer and contains a binder resin, a charge transport material, and metal oxide particles,
   in which, in a case where a cross section of the charge transport layer is observed, a proportion of single particles of the metal oxide particles to a total of the single particles and aggregated particles of the metal oxide particles is 60% by number or more.
<2> According to a second aspect of the present invention, there is provided the electrophotographic photoreceptor according to <1>,
   in which the proportion of the single particles of the metal oxide particles may be 70% by number or more.
<3> According to a third aspect of the present invention, there is provided the electrophotographic photoreceptor according to <1> or <2>,
   in which, in the case where the cross section of the charge transport layer is observed, a proportion of a total area of the single particles and the aggregated particles of the metal oxide particles to an area of an entire observed cross section may be 60% by area or more and 95% by area or less.
<4> According to a fourth aspect of the present invention, there is provided the electrophotographic photoreceptor according to any one of <1> to <3>,
   in which the metal oxide particles may be silica particles.
<5> According to a fifth aspect of the present invention, there is provided the electrophotographic photoreceptor according to any one of <1> to <4>,
   in which, in the metal oxide particles, an average circularity may be 0.7 or more and a degree of hydrophobicity may be 60% or more.
<6> According to a sixth aspect of the present invention, there is provided the electrophotographic photoreceptor according to <5>,
   in which, in the metal oxide particles, the average circularity may be 0.8 or more and the degree of hydrophobicity may be 60% or more.
<7> According to a seventh aspect of the present invention, there is provided the electrophotographic photoreceptor according to any one of <1> to <6>,
   in which a light transmittance T of the charge transport layer may be 80% or more.
<8> According to an eighth aspect of the present invention, there is provided the electrophotographic photoreceptor according to any one of <1> to <7>, further including:
   an inorganic protective layer that is disposed on the charge transport layer.
<9> According to a ninth aspect of the present invention, there is provided a process cartridge including:
   the electrophotographic photoreceptor according to any one of <1> to <8>,
   in which the process cartridge is attachable to and detachable from an image forming apparatus.
<10> According to a tenth aspect of the present invention, there is provided an image forming apparatus including:
   the electrophotographic photoreceptor according to any one of <1> to <8>;
   a charging device that charges a surface of the electrophotographic photoreceptor;
   an electrostatic latent image forming device that forms an electrostatic latent image on the charged surface of the electrophotographic photoreceptor;
   a developing device that develops the electrostatic latent image formed on the surface of the electrophotographic photoreceptor with a developer containing a toner to form a toner image; and
   a transfer device that transfers the toner image to a surface of a recording medium.

According to <1>, there is provided an electrophotographic photoreceptor including a conductive substrate, a charge generation layer that is disposed on the conductive substrate, and a charge transport layer that is disposed on the charge generation layer and contains a binder resin, a charge transport material, and metal oxide particles, in which the electrophotographic photoreceptor has excellent abrasion resistance and electrical properties, as compared with a case where, when a cross section of the charge transport layer is observed, a proportion of single particles of the metal oxide particles to a total of the single particles and aggregated particles of the metal oxide particles is less than 60% by number.

According to <2>, there is provided an electrophotographic photoreceptor having excellent abrasion resistance and electrical properties, as compared with a case where the proportion of the single particles of the metal oxide particles is less than 70% by number.

According to <3>, there is provided an electrophotographic photoreceptor having excellent abrasion resistance and electrical properties, as compared with a case where, when the cross section of the charge transport layer is observed, a proportion of a total area of the single particles and the aggregated particles of the metal oxide particles to an area of an entire observed cross section is less than 60% by area or more than 95% by area.

According to <4>, there is provided an electrophotographic photoreceptor having excellent abrasion resistance and electrical properties, as compared with a case where the metal oxide particles are not silica particles.

According to <5> or <6>, there is provided an electrophotographic photoreceptor having excellent abrasion resistance and electrical properties, as compared with a case where the average circularity of the metal oxide particles is less than 0.7 or the degree of hydrophobicity thereof is less than 60%, or a case where the average circularity of the metal oxide particles is less than 0.8 or the degree of hydrophobicity thereof is less than 60%.

According to <7>, there is provided an electrophotographic photoreceptor having excellent abrasion resistance and electrical properties, as compared with a case where the light transmittance T of the charge transport layer is less than 80%.

According to <8>, there is provided an electrophotographic photoreceptor including a conductive substrate, a charge generation layer that is disposed on the conductive substrate, and a charge transport layer that is disposed on the charge generation layer and contains a binder resin, a charge transport material, and metal oxide particles, in which the electrophotographic photoreceptor has excellent cracking prevention in an inorganic protective layer and electrical properties, as compared with a case where, when a cross section of the charge transport layer is observed, a proportion of single particles of the metal oxide particles to a total of the single particles and aggregated particles of the metal oxide particles is less than 60% by number.

According to <9> or <10>, there is provided a process cartridge or an image forming apparatus, each of which includes an electrophotographic photoreceptor including a conductive substrate, a charge generation layer that is disposed on the conductive substrate, and a charge transport layer that is disposed on the charge generation layer and contains a binder resin, a charge transport material, and metal oxide particles, in which the electrophotographic photoreceptor has excellent abrasion resistance and electrical properties, as compared with a case of adopting an electrophotographic photoreceptor in which, in a case where a cross section of the charge transport layer is observed, a proportion of single particles of the metal oxide particles to a total of the single particles and aggregated particles of the metal oxide particles is less than 60% by number.

### BRIEF DESCRIPTION OF THE DRAWINGS

Exemplary embodiment(s) of the present invention will be described in detail based on the following figures, wherein:
Fig. 1 is a partial cross-sectional view showing an example of a layer configuration of an electrophotographic photoreceptor according to the present exemplary embodiment;
Fig. 2 is a view schematically showing the configuration of an example of an image forming apparatus according to the present exemplary embodiment; and
Fig. 3 is a view schematically showing a configuration of another example of the image forming apparatus according to the present exemplary embodiment.

### DETAILED DESCRIPTION OF THE INVENTION

Hereinafter, exemplary embodiments of the present invention will be described. The following descriptions and examples merely illustrate the exemplary embodiments, and do not limit the scope of the present invention.

In the present specification, a numerical range described using "to" represents a range including numerical values listed before and after "to" as the minimum value and the maximum value respectively.

Regarding the numerical ranges described in stages in the present specification, the upper limit or lower limit of a numerical range may be replaced with the upper limit or lower limit of another numerical range described in stages. Furthermore, in the present specification, the upper limit or lower limit of a numerical range may be replaced with values described in examples.

In the present specification, the term "step" includes not only an independent step but a step that is not clearly distinguished from other steps as long as the purpose of the step is achieved.

In the present specification, in a case where an exemplary embodiment is described with reference to drawings, the configuration of the exemplary embodiment is not limited to the configuration shown in the drawings. In addition, the sizes of members in each drawing are conceptual and do not limit the relative relationship between the sizes of the members.

In the present specification, each component may include a plurality of corresponding substances. In a case where the amount of each component in a composition is mentioned in the present specification, and there are two or more kinds of substances corresponding to each component in the composition, unless otherwise specified, the amount of each component means the total amount of two or more kinds of the substances present in the composition.

In the present specification, each component may include two or more kinds of corresponding particles. In a case where there are two or more kinds of particles corresponding to each component in a composition, unless otherwise specified, the particle size of each component means a value for a mixture of two or more kinds of the particles present in the composition.

In the present specification, the term "axial direction" of an electrophotographic photoreceptor denotes a direction in which a rotation axis of the electrophotographic photoreceptor extends, and the term "circumferential direction" of the electrophotographic photoreceptor denotes a rotation direction of the electrophotographic photoreceptor.

### <Electrophotographic Photoreceptor>

The electrophotographic photoreceptor (hereinafter, also referred to as "photoreceptor") according to the present exemplary embodiment includes a conductive substrate, a charge generation layer, and a charge transport layer.

The charge generation layer is provided on the conductive substrate.

The charge transport layer contains a binder resin, a charge transport material, and metal oxide particles.

In a case where a cross section of the charge transport layer is observed, a proportion of single particles of the metal oxide particles to the total of the single particles and aggregated particles of the metal oxide particles is 60% by number or more.

With the above-described configuration, the photoreceptor according to the present exemplary embodiment is an electrophotographic photoreceptor having excellent abrasion resistance and electrical properties. The reason is presumed as follows.

In metal oxide particles, single particles are likely to aggregate with each other in the charge transport layer, that causes an increase in particle diameter and poor dispersion in the charge transport layer. Therefore, in the charge transport layer, a decrease in light transmittance due to light scattering and a variation in hardness of a surface of the charge transport layer occur. As a result, abrasion resistance and electrical properties as a photoreceptor are deteriorated.

Therefore, in the photoreceptor according to the present exemplary embodiment, the proportion of the single particles of the metal oxide particles is set to 60% by number as described above. That is, the metal oxide particles are dispersed in a state of having a small particle diameter and being close to uniform, without being aggregated in the charge transport layer. As a result, the scattering of light in the charge transport layer can be suppressed, and a decrease in light transmittance can be suppressed.

In addition, the metal oxide particles exhibiting a filler effect are dispersed on the surface of the charge transport layer in a state of having a small particle diameter and being close to uniform. As a result, the variation in hardness of the surface of the charge transport layer can be suppressed.

Due to the above-described reasons, it is presumed that the photoreceptor according to the present exemplary embodiment has excellent abrasion resistance and electrical properties.

Hereinafter, the photoreceptor according to the present exemplary embodiment will be described in detail.

Fig. 1 is a partial cross-sectional view schematically showing an example of a layer configuration of the photoreceptor according to the present exemplary embodiment. A photoreceptor 10A shown in Fig. 1 includes a lamination-type photosensitive layer.

The photoreceptor 10A has a structure in which an undercoat layer 2, a charge generation layer 3, a charge transport layer 4, and an inorganic protective layer 6 are laminated in this order on a conductive substrate 1, and the charge generation layer 3 and the charge transport layer 4 constitute a photosensitive layer 5 (so-called function separation-type photosensitive layer).

The photoreceptor 10A may include an interlayer (not shown) between the undercoat layer 2 and the charge generation layer 3. The undercoat layer 2 may or may not be provided. The inorganic protective layer 6 may or may not be provided.

Hereinafter, each layer of the photoreceptor will be described in detail. However, each layer of the photoreceptor will be described without a reference numeral.

### [Conductive Substrate]

Examples of the conductive substrate include metal plates, metal drums, metal belts, or the like, containing a metal (such as aluminum, copper, zinc, chromium, nickel, molybdenum, vanadium, indium, gold, and platinum) or an alloy (such as stainless steel). In addition, examples of the conductive substrate also include paper, a resin film, a belt, or the like, that is obtained by being coated, vapor-deposited, or laminated with a conductive compound (such as a conductive polymer and indium oxide), a metal (such as aluminum, palladium, and gold) or an alloy. Here, the term "conductive" denotes that a volume resistivity is less than 10¹³ Ω·cm.

In a case where the electrophotographic photoreceptor is used in a laser printer, for example, it is preferable that a surface of the conductive substrate is roughened such that a centerline average roughness Ra thereof is 0.04 µm or more and 0.5 µm or less for the purpose of suppressing interference fringes from occurring in a case of irradiation with laser beams. In a case where incoherent light is used as a light source, roughening of the surface to prevent the interference fringes is not particularly necessary, and it is appropriate for longer life because occurrence of defects due to the roughness of the surface of the conductive substrate is suppressed.

Examples of the roughening method include wet honing performed by suspending an abrasive in water and spraying the suspension to the conductive substrate, centerless grinding performed by pressure-welding the conductive substrate against a rotating grindstone and continuously grinding the conductive substrate, and an anodizing treatment.

Examples of the roughening method also include a method of dispersing conductive or semi-conductive powder in a resin without roughening the surface of the conductive substrate to form a layer on the surface of the conductive substrate, and performing roughening using the particles dispersed in the layer.

The roughening treatment by anodization is a treatment of forming an oxide film on the surface of the conductive substrate by carrying out anodization in an electrolytic solution using a conductive substrate made of a metal (for example, aluminum) as an anode. Examples of the electrolytic solution include a sulfuric acid solution and an oxalic acid solution. However, a porous anodized film formed by the anodization is chemically active in a natural state, is easily contaminated, and has a large resistance fluctuation depending on the environment. Therefore, for example, it is preferable that a sealing treatment is performed on the porous anodized film so that micropores of the oxide film are closed by volume expansion due to a hydration reaction in pressurized steam or boiling water (a metal salt such as nickel may be added thereto) for a change into a more stable a hydrous oxide.

A film thickness of the anodized film is, for example, preferably 0.3 µm or more and 15 µm or less. In a case where the film thickness is within the above-described range, barrier properties against injection tend to be exhibited, and an increase in the residual potential due to repeated use tends to be suppressed.

The conductive substrate may be subjected to a treatment with an acidic treatment liquid or a boehmite treatment.

The treatment with an acidic treatment liquid is carried out, for example, as follows. First, an acidic treatment liquid containing phosphoric acid, chromic acid, and hydrofluoric acid is prepared. As a blending proportion of the phosphoric acid, chromic acid, and hydrofluoric acid to the acidic treatment liquid, for example, a concentration of the phosphoric acid may be in a range of 10% by mass or more and 11% by mass or less, a concentration of the chromic acid may be in a range of 3% by mass or more and 5% by mass or less, and a concentration of the hydrofluoric acid may be in a range of 0.5% by mass or more and 2% by mass or less, and a concentration of all of these acids may be in a range of 13.5% by mass or more and 18% by mass or less. A treatment temperature is, for example, preferably 42°C or higher and 48°C or lower. A film thickness of the coating film is, for example, preferably 0.3 µm or more and 15 µm or less.

The boehmite treatment is carried out, for example, by dipping the base material in pure water at 90°C or higher and 100°C or lower for 5 minutes to 60 minutes, or by bringing the base material into contact with heated steam at 90°C or higher and 120°C or lower for 5 minutes to 60 minutes. A film thickness of the coating film is, for example, preferably 0.1 µm or more and 5 µm or less. The coating film may be further subjected to an anodizing treatment using an electrolytic solution having low film solubility, such as adipic acid, boric acid, a borate, a phosphate, a phthalate, a maleate, a benzoate, a tartrate, or a citrate.

### (Undercoat Layer)

The undercoat layer is, for example, a layer containing inorganic particles and a binder resin.

Examples of the inorganic particles include inorganic particles having a powder resistance (volume resistivity) of 10² Ω·cm or more and 10¹¹ Ω·cm or less.

Among the above, as the inorganic particles having the above-described resistance value, for example, metal oxide particles such as tin oxide particles, titanium oxide particles, zinc oxide particles, and zirconium oxide particles may be used, and zinc oxide particles are particularly preferable.

A specific surface area of the inorganic particles, measured by a BET method, may be, for example, 10 m²/g or more.

A volume-average particle diameter of the inorganic particles may be 50 nm or more and 2,000 nm or less (for example, preferably 60 nm or more and 1,000 nm or less).

A content of the inorganic particles is, for example, preferably 10% by mass or more and 80% by mass or less, and more preferably 40% by mass or more and 80% by mass or less with respect to the binder resin.

The inorganic particles may be subjected to a surface treatment. As the inorganic particles, two or more kinds of inorganic particles subjected to different surface treatments or two or more kinds of inorganic particles having different particle diameters may be used in a form of a mixture.

Examples of a surface treatment agent include a silane coupling agent, a titanate-based coupling agent, an aluminum-based coupling agent, and a surfactant. In particular, for example, a silane coupling agent is preferable, and a silane coupling agent having an amino group is more preferable.

Examples of the silane coupling agent having an amino group include 3-aminopropyltriethoxysilane, N-2-(aminoethyl)-3-aminopropyltrimethoxysilane, N-2-(aminoethyl)-3-aminopropylmethyldimethoxysilane, and N,N-bis(2-hydroxyethyl)-3-aminopropyltriethoxysilane; but the present invention is not limited thereto.

The silane coupling agent may be used in a form of a mixture of two or more kinds thereof. For example, the silane coupling agent having an amino group and other silane coupling agents may be used in combination. Examples of the other silane coupling agents include vinyltrimethoxysilane, 3-methacryloxypropyl-tris(2-methoxyethoxy)silane, 2-(3,4-epoxycyclohexyl)ethyltrimethoxysilane, 3-glycidoxypropyltrimethoxysilane, vinyltriacetoxysilane, 3-mercaptopropyltrimethoxysilane, 3-aminopropyltriethoxysilane, N-2-(aminoethyl)-3-aminopropyltrimethoxysilane, N-2-(aminoethyl)-3-aminopropylmethyldimethoxysilane, N,N-bis(2-hydroxyethyl) -3-aminopropyltriethoxysilane, and 3-chloropropyltrimethoxysilane; but the present invention is not limited thereto.

A surface treatment method using the surface treatment agent may be any method as long as the method is a known method, and any of a dry method or a wet method may be used.

A treatment amount of the surface treatment agent is, for example, preferably 0.5% by mass or more and 10% by mass or less with respect to the inorganic particles.

Here, for example, the undercoat layer may contain an electron-accepting compound (acceptor compound) together with the inorganic particles from the viewpoint of enhancing long-term stability of electrical properties and carrier blocking properties.

Examples of the electron-accepting compound include electron-transporting substances, for example, a compound having an anthraquinone structure; a quinone-based compound such as chloranil and bromanil; a tetracyanoquinodimethane-based compound; a fluorenone compound such as 2,4,7-trinitrofluorenone and 2,4,5,7-tetranitro-9-fluorenone; an oxadiazole-based compound such as 2-(4-biphenyl)-5-(4-t-butylphenyl)-1,3,4-oxadiazole, 2,5-bis(4-naphthyl)-1,3,4-oxadiazole, and 2,5-bis(4-diethylaminophenyl)-1,3,4-oxadiazole; a xanthone-based compound; a thiophene compound; a diphenoquinone compound such as 3,3',5,5'-tetra-t-butyldiphenoquinone; and a benzophenone compound.

In particular, as the electron-accepting compound, for example, a compound having an anthraquinone structure is preferable. As the compound having an anthraquinone structure, for example, a hydroxyanthraquinone compound, an aminoanthraquinone compound, or an aminohydroxyanthraquinone compound is preferable; and specifically, anthraquinone, alizarin, quinizarin, anthrarufin, purpurin, or a derivative thereof is preferable.

The electron-accepting compound may be contained in the undercoat layer in a state of being dispersed with the inorganic particles, or in a state of being attached to the surface of the inorganic particles.

Examples of a method of attaching the electron-accepting compound to the surface of the inorganic particles include a dry method and a wet method.

The dry method is, for example, a method of attaching the electron-accepting compound to the surface of the inorganic particles by adding the electron-accepting compound dropwise to the inorganic particles directly or by dissolving the electron-accepting compound in an organic solvent while stirring the inorganic particles with a mixer having a large shearing force and spraying the mixture together with dry air or nitrogen gas. For example, the dropwise addition or spraying of the electron-accepting compound may be performed at a temperature equal to or lower than a boiling point of the solvent. After the dropwise addition or spraying of the electron-accepting compound, the mixture may be further baked at 100°C or higher. The baking is not particularly limited as long as the temperature and the time are adjusted such that electrophotographic characteristics can be obtained.

The wet method is, for example, a method of attaching the electron-accepting compound to the surface of the inorganic particles by adding the electron-accepting compound to inorganic particles while dispersing the inorganic particles in a solvent by performing using a stirrer, an ultrasonic disperser, a sand mill, an attritor, or a ball mill, stirring or dispersing the mixture, and removing the solvent. The solvent removing method is carried out by, for example, filtration or distillation so that the solvent is distilled off. After removal of the solvent, the mixture may be further baked at 100°C or higher. The baking is not particularly limited as long as the temperature and the time are adjusted such that electrophotographic characteristics can be obtained. In the wet method, the moisture contained in the inorganic particles may be removed before the electron-accepting compound is added, and examples thereof include a method of removing the moisture while stirring and heating the inorganic particles in a solvent and a method of removing the moisture by azeotropically boiling the inorganic particles with a solvent.

The electron-accepting compound may be attached before or after the inorganic particles are subjected to the surface treatment with the surface treatment agent or simultaneously with the surface treatment with the surface treatment agent.

A content of the electron-accepting compound may be, for example, 0.01% by mass or more and 20% by mass or less, preferably 0.01% by mass or more and 10% by mass or less with respect to the inorganic particles.

Examples of the binder resin used for the undercoat layer include a known polymer compound such as an acetal resin (such as polyvinyl butyral), a polyvinyl alcohol resin, a polyvinyl acetal resin, a casein resin, a polyamide resin, a cellulose resin, gelatin, a polyurethane resin, a polyester resin, an unsaturated polyester resin, a methacrylic resin, an acrylic resin, a polyvinyl chloride resin, a polyvinyl acetate resin, a vinyl chloride-vinyl acetate-maleic anhydride resin, a silicone resin, a silicone-alkyd resin, a urea resin, a phenol resin, a phenol-formaldehyde resin, a melamine resin, a urethane resin, an alkyd resin, and an epoxy resin; a zirconium chelate compound; a titanium chelate compound; an aluminum chelate compound; a titanium alkoxide compound; an organic titanium compound; and a known material such as a silane coupling agent.

Examples of the binder resin used for the undercoat layer also include a charge-transporting resin having a charge-transporting group, and a conductive resin (for example, polyaniline or the like).

Among the above, as the binder resin used for the undercoat layer, for example, a resin insoluble in a coating solvent of an upper layer is suitable; and a resin obtained by a reaction between at least one resin selected from the group consisting of a thermosetting resin such as a urea resin, a phenol resin, a phenol-formaldehyde resin, a melamine resin, a urethane resin, an unsaturated polyester resin, an alkyd resin, or an epoxy resin; a polyamide resin, a polyester resin, a polyether resin, a methacrylic resin, an acrylic resin, a polyvinyl alcohol resin, and a polyvinyl acetal resin, and a curing agent is particularly suitable.

In a case where these binder resins are used in combination of two or more kinds thereof, a mixing proportion thereof is set as necessary.

The undercoat layer may contain various additives for improving the electrical properties, the environmental stability, and the image quality.

Examples of the additive include known materials, for example, an electron-transporting pigment such as a polycyclic condensed pigment or an azo-based pigment, a zirconium chelate compound, a titanium chelate compound, an aluminum chelate compound, a titanium alkoxide compound, an organic titanium compound, and a silane coupling agent. The silane coupling agent is used for the surface treatment of the inorganic particles as described above, but may be further added to the undercoat layer as the additive.

Examples of the silane coupling agent as the additive include vinyltrimethoxysilane, 3-methacryloxypropyl-tris(2-methoxyethoxy)silane, 2-(3,4-epoxycyclohexyl)ethyltrimethoxysilane, 3-glycidoxypropyltrimethoxysilane, vinyltriacetoxysilane, 3-mercaptopropyltrimethoxysilane, 3-aminopropyltriethoxysilane, N-2-(aminoethyl)-3-aminopropyltrimethoxysilane, N-2-(aminoethyl)-3-aminopropylmethyldimethoxysilane, N,N-bis(2-hydroxyethyl) -3-aminopropyltriethoxysilane, and 3-chloropropyltrimethoxysilane.

Examples of the zirconium chelate compound include zirconium butoxide, ethyl zirconium acetoacetate, zirconium triethanolamine, acetylacetonate zirconium butoxide, ethyl zirconium butoxide acetoacetate, zirconium acetate, zirconium oxalate, zirconium lactate, zirconium phosphonate, zirconium octanoate, zirconium naphthenate, zirconium laurate, zirconium stearate, zirconium isostearate, zirconium butoxide methacrylate, stearate zirconium butoxide, and isostearate zirconium butoxide.

Examples of the titanium chelate compound include tetraisopropyl titanate, tetranormal butyl titanate, a butyl titanate dimer, tetra(2-ethylhexyl) titanate, titanium acetylacetonate, polytitanium acetylacetonate, titanium octylene glycolate, titanium lactate ammonium salt, titanium lactate, titanium lactate ethyl ester, titanium triethanol aminate, and polyhydroxy titanium stearate.

Examples of the aluminum chelate compound include aluminum isopropylate, monobutoxyaluminum diisopropylate, aluminum butyrate, diethylacetoacetate aluminum diisopropylate, and aluminum tris(ethylacetoacetate).

These additives may be used alone or in a form of a mixture or a polycondensate of a plurality of compounds.

The undercoat layer may have, for example, a Vickers hardness of 35 or more.

For example, the surface roughness (ten-point average roughness) of the undercoat layer may be adjusted to 1/2 from 1/(4n) (n represents a refractive index of an upper layer) of a laser wavelength λ for exposure to be used to suppress moire fringes.

Resin particles or the like may be added to the undercoat layer to adjust the surface roughness. Examples of the resin particles include silicone resin particles and crosslinked polymethyl methacrylate resin particles. In addition, the surface of the undercoat layer may be polished to adjust the surface roughness. Examples of a polishing method include buff polishing, a sandblast treatment, wet honing, and a grinding treatment.

The formation of the undercoat layer is not particularly limited, and a known forming method is used. For example, a coating film of a coating solution for forming the undercoat layer, in which the above-described components are added to a solvent, is formed, and the coating film is dried and then heated as necessary.

Examples of the solvent for preparing the coating solution for forming the undercoat layer include known organic solvents such as an alcohol-based solvent, an aromatic hydrocarbon solvent, a halogenated hydrocarbon solvent, a ketone-based solvent, a ketone alcohol-based solvent, an ether-based solvent, and an ester-based solvent.

Specific examples of the solvent include typical organic solvents such as methanol, ethanol, n-propanol, iso-propanol, n-butanol, benzyl alcohol, methyl cellosolve, ethyl cellosolve, acetone, methyl ethyl ketone, cyclohexanone, methyl acetate, ethyl acetate, n-butyl acetate, dioxane, tetrahydrofuran, methylene chloride, chloroform, chlorobenzene, and toluene.

Examples of the method of dispersing the inorganic particles in a case of preparing the coating solution for forming the undercoat layer include known methods such as a roll mill, a ball mill, a vibration ball mill, an attritor, a sand mill, a colloid mill, and a paint shaker.

Examples of the method of coating the conductive substrate with the coating solution for forming the undercoat layer include typical coating methods such as a blade coating method, a wire bar coating method, a spray coating method, a dip coating method, a bead coating method, an air knife coating method, and a curtain coating method.

A film thickness of the undercoat layer is set to, for example, preferably 15 µm or more and more preferably in a range of 20 µm or more and 50 µm or less.

### (Interlayer)

Although not shown in the drawings, an interlayer may be further provided between the undercoat layer and the photosensitive layer.

The interlayer is, for example, a layer containing a resin. Examples of the resin used for the interlayer include polymer compounds such as an acetal resin (for example, polyvinyl butyral or the like), a polyvinyl alcohol resin, a polyvinyl acetal resin, a casein resin, a polyamide resin, a cellulose resin, gelatin, a polyurethane resin, a polyester resin, a methacrylic resin, an acrylic resin, a polyvinyl chloride resin, a polyvinyl acetate resin, a vinyl chloride-vinyl acetate-maleic anhydride resin, a silicone resin, a silicone-alkyd resin, a phenol-formaldehyde resin, and a melamine resin.

The interlayer may be a layer containing an organometallic compound. Examples of the organometallic compound used for the interlayer include organometallic compounds containing a metal atom such as zirconium, titanium, aluminum, manganese, and silicon.

The compounds used for the interlayer may be used alone or in a form of a mixture or a polycondensate of a plurality of compounds.

Among the above, for example, it is preferable that the interlayer is a layer containing an organometallic compound containing a zirconium atom or a silicon atom.

The formation of the interlayer is not particularly limited, and a known forming method is used. For example, a coating film of a coating solution for forming the interlayer, in which the above-described components are added to a solvent, is formed, and the coating film is dried and then heated as necessary.

Examples of the coating method of forming the interlayer include typical methods such as a dip coating method, a push-up coating method, a wire bar coating method, a spray coating method, a blade coating method, an air knife coating method, and a curtain coating method.

A film thickness of the interlayer is set to, for example, preferably in a range of 0.1 µm or more and 3 µm or less. The interlayer may be used as the undercoat layer.

### (Charge Generation Layer)

A charge generation layer is, for example, a layer containing a charge generation material and a binder resin. In addition, the charge generation layer may be a deposition layer of the charge generation material. For example, the deposition layer of the charge generation material is suitable in a case where an incoherent light source such as a light emitting diode (LED) and an organic electro-luminescence (EL) image array is used.

Examples of the charge generation material include an azo pigment such as a bisazo pigment and a trisazo pigment; a fused ring aromatic pigment such as dibromoanthanthrone; a perylene pigment; a pyrrolopyrrole pigment; a phthalocyanine pigment; zinc oxide; and trigonal selenium.

Among the above, for example, a metal phthalocyanine pigment or a metal-free phthalocyanine pigment is preferably used as the charge generation material, in order to deal with laser exposure in a near-infrared region. Specifically, for example, hydroxy gallium phthalocyanine, chlorogallium phthalocyanine, dichlorotin phthalocyanine, or titanyl phthalocyanine is more preferable.

On the other hand, for example, a fused ring aromatic pigment such as dibromoanthanthrone; a thioindigo-based pigment; a porphyrazine compound; zinc oxide; trigonal selenium; or a bisazo pigment is preferable as the charge generation material in order to deal with laser exposure in a near-ultraviolet region.

The above-described charge generation material may be used even in a case where a non-coherent light source such as an LED having a central wavelength of light emission in a range of 450 nm or more and 780 nm or less and an organic EL image array is used.

In a case where an n-type semiconductor such as a fused ring aromatic pigment, a perylene pigment, and an azo pigment is used as the charge generation material, a dark current is unlikely to be generated, and image defects referred to as black spots can be suppressed even in a case in which a thin film is used as the photosensitive layer.

The n-type is determined by the polarity of the flowing photocurrent using a typically used time-of-flight method, and a material in which electrons more easily flow as carriers than positive holes is determined as the n-type.

The binder resin used for the charge generation layer is selected from a wide range of insulating resins, and the binder resin may be selected from organic photoconductive polymers such as poly-N-vinylcarbazole, polyvinyl anthracene, polyvinylpyrene, and polysilane.

Examples of the binder resin include a polyvinyl butyral resin, a polyarylate resin (polycondensate of bisphenols and aromatic divalent carboxylic acid, or the like), a polycarbonate resin, a polyester resin, a phenoxy resin, a vinyl chloride-vinyl acetate copolymer, a polyamide resin, an acrylic resin, a polyacrylamide resin, a polyvinylpyridine resin, a cellulose resin, a urethane resin, an epoxy resin, casein, a polyvinyl alcohol resin, and a polyvinylpyrrolidone resin. Here, the term "insulating" means that a volume resistivity is 10¹³ Ω·cm or more.

The binder resins may be used alone or in a form of a mixture of two or more kinds thereof.

A blending ratio between the charge generation material and the binder resin is, for example, preferably in a range of 10: 1 to 1:10 in terms of mass ratio.

The charge generation layer may also contain other known additives.

The formation of the charge generation layer is not particularly limited, and a known forming method is used. For example, a coating film of a coating solution for forming the charge generation layer, in which the above-described components are added to a solvent, is formed, and the coating film is dried and then heated as necessary. The charge generation layer may be formed by a vapor deposition of the charge generation material. For example, the formation of the charge generation layer by the vapor deposition is particularly preferable in a case where the fused ring aromatic pigment or the perylene pigment is used as the charge generation material.

Examples of the solvent for preparing the coating solution for forming the charge generation layer include methanol, ethanol, n-propanol, n-butanol, benzyl alcohol, methyl cellosolve, ethyl cellosolve, acetone, methyl ethyl ketone, cyclohexanone, methyl acetate, n-butyl acetate, dioxane, tetrahydrofuran, methylene chloride, chloroform, chlorobenzene, and toluene. The solvents are used alone or in a form of a mixture of two or more kinds thereof.

As a method of dispersing particles (for example, the charge generation material) in the coating solution for forming the charge generation layer, for example, a media disperser such as a ball mill, a vibration ball mill, an attritor, a sand mill, and a horizontal sand mill, or a medialess disperser such as a stirrer, an ultrasonic disperser, a roll mill, and a high-pressure homogenizer is used. Examples of the high-pressure homogenizer include a collision type high-pressure homogenizer in which a dispersion liquid is dispersed by a liquid-liquid collision or a liquid-wall collision in a high-pressure state, and a penetration type high-pressure homogenizer in which a dispersion liquid is dispersed by causing the dispersion liquid to penetrate through a micro-flow path in a high-pressure state.

During the dispersion, it is effective to set an average particle diameter of the charge generation material in the coating solution for forming the charge generation layer to 0.5 µm or less, for example, preferably 0.3 µm or less and more preferably 0.15 µm or less.

Examples of the method of coating the undercoat layer (or the interlayer) with the coating solution for forming the charge generation layer include typical methods such as a blade coating method, a wire bar coating method, a spray coating method, a dip coating method, a bead coating method, an air knife coating method, and a curtain coating method.

A film thickness of the charge generation layer is set to, for example, preferably in a range of 0.1 µm or more and 5.0 µm or less and more preferably in a range of 0.2 µm or more and 2.0 µm or less.

### [Charge Transport Layer]

The charge transport layer is a layer containing a binder resin, a charge transport material, and metal oxide particles.

The charge transport layer may be a layer containing a binder resin, a polymer charge transport material, and metal oxide particles.

In the photoreceptor according to the present exemplary embodiment, in a case where a cross section of the charge transport layer is observed, a proportion of single particles of the metal oxide particles to the total of the single particles and aggregated particles of the metal oxide particles is 60% by number or more.

In a case where the proportion of the single particles of the metal oxide particles is less than 60% by number, the aggregated particles inhibit charge transfer, and the conductivity of the charge transport layer decreases.

The proportion of the single particles of the metal oxide particles is, for example, preferably 60% by number or more, more preferably 80% by number or more, and still more preferably 90% by number or more.

In a case where the proportion of the single particles of the metal oxide particles satisfies the above-described range when the cross section of the charge transport layer is observed, both the abrasion resistance and the electrical properties of the photoreceptor are excellent.

Here, the "% by number" as the proportion of the single particles of the metal oxide particles is calculated by observing the cross section of the charge transport layer by the following method.

A sample piece of the charge transport layer, that has been cut along a thickness direction, is obtained by a cryomicrotome method.

A cross section of the sample piece is observed with a scanning electron microscope at a magnification of 20,000 times.

The number of single particles and aggregated particles of the metal oxide particles in the observation region is counted.

Here, the single particles of the metal oxide particles are particles in which primary particles of the metal oxide particles are observed without coming into contact with or overlapping with other particles.

On the other hand, the aggregated particles of the metal oxide particles are particles in which the primary particles of the metal oxide particles are observed to be in contact with or overlap with other particles.

A proportion of the number of the single particles of the metal oxide particles to the total number of the single particles and the aggregated particles of the metal oxide particles in the observation region is calculated.

Next, the above-described operation is performed 5 times, and the calculated average value of the proportion of the number of the single particles of the metal oxide particles is calculated.

In the observation of the cross section of the sample piece, the metal oxide particles are identified based on the presence of constituent elements of the metal oxide particles (for example, in a case of silica particles, Si and O) by analysis with energy dispersive X-ray spectroscopy (EDX).

Examples of a method of allowing the metal oxide particles contained in the charge transport layer to satisfy the above-described range include a method of adjusting a temperature of a coating environment of a coating solution for forming the charge transport layer.

In addition, in the photoreceptor according to the present exemplary embodiment, in a case where the cross section of the charge transport layer is observed, a proportion of the total area of the single particles and the aggregated particles of the metal oxide particles to an area of the entire observed cross section is, for example, preferably 60% by area or more and 95% by area or less.

In a case where the "% by area" of the total of the metal oxide particles is less than 60% by area, the abrasion resistance of the charge transport layer is not sufficient.

In a case where the "% by area" of the single particles of the metal oxide particles is more than 95% by area, the metal oxide particles inhibit movement of charge, and the conductivity of the charge transport layer decreases.

The "% by area" of the single particles of the metal oxide particles is, for example, more preferably 65% by area or more and 92% by area or less, and still more preferably 70% by area or more and 90% by area or less.

Here, the "% by area" as the proportion of the single particles of the metal oxide particles is calculated by observing the cross section of the charge transport layer by the following method.

A sample piece of the charge transport layer, that has been cut along a thickness direction, is obtained by a cryomicrotome method.

A cross section of the sample piece is observed with a scanning electron microscope at a magnification of 20,000 times.

The total area of the single particles and the aggregated particles of the metal oxide particles in the observation region is calculated.

The single particles and the aggregated particles of the metal oxide particles are identified as described in the proportion of the single particles of the metal oxide particles.

A proportion of the total area of the single particles and the aggregated particles of the metal oxide particles to the area of the observation region is calculated.

Next, the above-described operation is performed 5 times, and the calculated average value of the proportion of the total area of the single particles and the aggregated particles of the metal oxide particles is calculated.

The metal oxide particles in the cross-sectional observation of the sample piece are also identified as described in the proportion of the single particles of the metal oxide particles.

### (Type of Metal Oxide Particles)

Examples of the metal oxide particles used in the charge transport layer include silica particles, alumina particles, and titanium oxide particles.

Among the above, from the viewpoint of suppressing the deterioration in electrical properties of the photoreceptor, the metal oxide particles are, for example, preferably silica particles.

Examples of the silica particles include dry silica particles and wet silica particles.

Examples of the dry silica particles include combustion silica (fumed silica) and explosion silica. The combustion silica is obtained by combustion of a silane compound. The explosion silica is obtained by explosively combusting metal silicon powder.

Examples of the wet silica particles include sedimentation silica, gel silica particles, colloidal silica particles (silica sol particles), and sol-gel silica particles.

The sedimentation silica and the gel silica particles are obtained by a neutralization reaction between sodium silicate and a mineral acid. A silica synthesized and aggregated under alkaline conditions is referred to as the sedimentation silica, and a silica synthesized and aggregated under acidic conditions is referred to as the gel silica particles.

The colloidal silica particles (silica sol particles) are obtained by polymerizing acidic silicate in an alkaline manner.

The sol-gel silica particles are obtained by hydrolysis of an organic silane compound (for example, alkoxysilane).

For example, the silica particles may have a surface subjected to a surface treatment with a hydrophobic agent.

In this manner, the number of silanol groups on the surface of the silica particles is reduced, and the occurrence of the residual potential is easily suppressed.

Examples of the hydrophobic agent include known silane compounds such as chlorosilane, alkoxysilane, and silazane.

Among the above, from the viewpoint of easily suppressing the generation of the residual potential, for example, a silane compound having a trimethylsilyl group, a decylsilyl group, or a phenylsilyl group is desirable as the hydrophobic agent. That is, for example, the surface of the silica particles may have a trimethylsilyl group, a decylsilyl group, or a phenylsilyl group.

Examples of the silane compound having a trimethylsilyl group include trimethylchlorosilane, trimethylmethoxysilane, and 1,1,1,3,3,3-hexamethyldisilazane.

Examples of the silane compound having a decylsilyl group include decyltrichlorosilane, decyldimethylchlorosilane, and decyltrimethoxysilane.

Examples of the silane compound having a phenyl group include triphenylmethoxysilane and triphenylchlorosilane.

### -Average Circularity of Metal Oxide Particles-

In the photoreceptor according to the present exemplary embodiment, for example, it is preferable that the metal oxide particles are dispersed in the charge transport layer in a state of having a small particle diameter and being close to uniform.

The metal oxide particles contained in the photoreceptor according to the present exemplary embodiment have an average circularity of, for example, preferably 0.7 or more, and more preferably 0.75 or more. The average circularity is, for example, still more preferably 0.8 or more.

In a case where the average circularity is 0.7 or more, an interparticle distance is likely to be uniform, and the particles are likely to be uniformly dispersed.

The average circularity of the metal oxide particles is calculated by the following method.

The average circularity of the metal oxide particles is determined by (Equivalent circular perimeter)/(Perimeter) [(Perimeter of circle having the same projected area as particle image)/(Perimeter of projected particle image)].

Specifically, the average circularity is a value measured by the following method.

A sample piece of the charge transport layer, that has been cut along a thickness direction, is obtained by a cryomicrotome method.

A cross section of the sample piece is observed with a scanning electron microscope at a magnification of 20,000 times.

The circularity of the primary particles of the metal oxide particles in the observation region is determined.

Next, the above-described operation is performed 5 times, and the calculated average value of the circularity of the primary particles of the metal oxide particles is calculated.

The metal oxide particles in the cross-sectional observation of the sample piece are also identified as described in the proportion of the single particles of the metal oxide particles.

### -Degree of Hydrophobicity of Metal Oxide Particles-

In the photoreceptor according to the present exemplary embodiment, in a case where the charge transport layer contains metal oxide particles having a small amount of OH groups, charges are not easily captured, and thus the electrical function of the charge transport layer is not easily deteriorated.

As an indicator indicating that the amount of OH groups is small, a degree of hydrophobicity of the metal oxide particles is, for example, preferably 60% or more, more preferably 62% or more, and still more preferably 65% or more.

In a case where the degree of hydrophobicity of the metal oxide particles is 60% or more, the amount of OH groups present in the particles serving as charge traps is small, and the inhibition of the function as a charge transport agent is suppressed.

Therefore, in a case where the average circularity and the degree of hydrophobicity of the metal oxide particles satisfy the above-described ranges, both the abrasion resistance and the electrical properties of the photoreceptor are improved.

Here, the silica particles as the metal oxide particles are generally subjected to a surface treatment with a hydrophobic agent in order to reduce the OH group remaining on the surface. However, in the silica particles, for example, silica particles produced by a sol-gel method have a porous structure, and thus the surface treatment agent is unlikely to permeate into an inside of pores, and a large number of OH groups remain in the inside of pores. Therefore, the silica particles are, for example, preferably subjected to a hydrophobic treatment with a hydrophobic agent.

The amount of OH groups of the metal oxide is determined by the degree of hydrophobicity.

The degree of hydrophobicity of the metal oxide particles is calculated by the following method.

5 g of the metal oxide particles are added to 100 mL of water. Methanol is added dropwise by 1 mL at a time, and the following values are set as the degree of hydrophobicity when the metal oxide particles are precipitated. [(Volume of dropped methanol)/ { (Volume of dropped methanol) + (Volume of water)}] × 100

In addition, as a method of separating the metal oxide particles from the photoreceptor, for example, a film peeled off from a substrate is dissolved in an organic solvent, and the solution is sieved to separate the particles.

### -Light Transmittance-

In the photoreceptor according to the present exemplary embodiment, for example, it is preferable that irradiated light is not likely to be scattered in the charge transport layer and is transmitted to the charge generation layer.

In the photoreceptor according to the present exemplary embodiment, a light transmittance T of the charge transport layer is, for example, preferably 80% or more.

In a case where the light transmittance T of the charge transport layer is less than 80%, the intensity of light transmitted through the charge transport layer and reaching the charge generation layer is insufficient, and the function as the photoreceptor is deteriorated.

In a case where the light transmittance T satisfies the above-described range, the metal oxide particles contained in the charge transport layer are dispersed in a state close to uniform. As described above, from the viewpoint of making it difficult for the light to be scattered in the layer and allowing the light to be transmitted to the charge generation layer, the light transmittance T of the charge transport layer is, for example, preferably 80% or more, more preferably 85% or more, and still more preferably 90% or more.

The light transmittance of the charge transport layer is calculated by the following method.

The coating solution for forming the charge transport layer is applied onto a polycarbonate sheet and dried to produce a laminate (polycarbonate sheet/composition layer), and the laminate is used as a measurement sample.

Using an ultraviolet-visible spectrophotometer, the light transmittance of the measurement sample in a thickness direction is measured at a wavelength of 730 to 830 nm. During the measurement, the light is incident from the polycarbonate sheet side. A light transmittance of only the polycarbonate sheet is also measured, and the transmittance of light incident on the composition layer and transmitted through the composition layer is obtained. An average value of the transmittances at every 10 nm at the wavelength of 730 nm to 830 nm is obtained.

Alternatively, a film of the charge transport layer is peeled off from a substrate, the film is attached to a glass plate, and the light transmittance is measured in the same manner as described above. In this case, the light is incident from the glass plate side, and a light transmittance of only the glass plate is also measured to obtain the measured value of the light transmittance of the charge transport layer alone.

### (Charge Transport Material)

Examples of the charge transport material include a quinone-based compound such as p-benzoquinone, chloranil, bromanil, and anthraquinone; a tetracyanoquinodimethane-based compound; a fluorenone compound such as 2,4,7-trinitrofluorenone; a xanthone-based compound; a benzophenone-based compound; a cyanovinyl-based compound; and an electron-transporting compound such as an ethylene-based compound. Examples of the charge transport material also include a positive hole-transporting compound such as a triarylamine-based compound, a benzidine-based compound, an arylalkane-based compound, an aryl-substituted ethylene-based compound, a stilbene-based compound, an anthracene-based compound, and a hydrazone-based compound. The charge transport materials may be used alone or in combination of two or more kinds thereof, but are not limited thereto.

From the viewpoint of charge mobility, for example, a triarylamine derivative represented by Structural Formula (a-1) or a benzidine derivative represented by Structural Formula (a-2) is preferable as the charge transport material.

In Structural Formula (a-1), Ar^{T1}, Ar^{T2}, and Ar^{T3} each independently represent a substituted or unsubstituted aryl group, -C₆H₄-C(R^{T4})=C(R^{T5})(R^{T6}), or -C₆H₄-CH=CH-CH=C(R^{T7})(R^{T8}). R^{T4}, R^{T5}, R^{T6}, R^{T7}, and R^{T8} each independently represent a hydrogen atom, a substituted or unsubstituted alkyl group, or a substituted or unsubstituted aryl group.

Examples of the substituent of each group described above include a halogen atom, an alkyl group having 1 or more and 5 or less carbon atoms, and an alkoxy group having 1 or more and 5 or less carbon atoms. In addition, examples of the substituent of each group described above also include a substituted amino group substituted with an alkyl group having 1 or more and 3 or less carbon atoms.

In Structural Formula (a-2), R^{T91} and R^{T92} each independently represent a hydrogen atom, a halogen atom, an alkyl group having 1 or more and 5 or less carbon atoms, or an alkoxy group having 1 or more and 5 or less carbon atoms. R^{T101}, R^{T102}, R^{T111}, and R^{T112} each independently represent a halogen atom, an alkyl group having 1 or more and 5 or less carbon atoms, an alkoxy group having 1 or more and 5 or less carbon atoms, an amino group substituted with an alkyl group having 1 or more and 2 or less carbon atoms, a substituted or unsubstituted aryl group, -C(R^{T12})-C(R^{T13})(R^{T14}), or -CH=CH-CH=C(R^{T15})(R^{T16}), in which R^{T12}, R^{T13}, R^{T14}, R^{T15}, and R^{T16} each independently represent a hydrogen atom, a substituted or unsubstituted alkyl group, or a substituted or unsubstituted aryl group. Tₘ₁, Tₘ₂, Tₙ₁, and Tₙ₂ each independently represent an integer of 0 or more and 2 or less.

Examples of the substituent of each group described above include a halogen atom, an alkyl group having 1 or more and 5 or less carbon atoms, and an alkoxy group having 1 or more and 5 or less carbon atoms. In addition, examples of the substituent of each group described above also include a substituted amino group substituted with an alkyl group having 1 or more and 3 or less carbon atoms.

Here, among the triarylamine derivative represented by Structural Formula (a-1) and the benzidine derivative represented by Structural Formula (a-2), for example, a triarylamine derivative having "-C₆H₄-CH=CH-CH=C(R^{T7})(R^{T8})" or a benzidine derivative having "-CH=CH-CH=C(R^{T15})(R^{T16})" is particularly preferable from the viewpoint of the charge mobility.

As the polymer charge transport material, known materials having charge transport properties, such as poly-N-vinylcarbazole and polysilane, are used. In particular, for example, a polyester-based polymer charge transport material is particularly preferable. The polymer charge transport material may be used alone or in combination of the binder resin.

Examples of the binder resin used for the charge transport layer include a polycarbonate resin, a polyester resin, a polyarylate resin, a methacrylic resin, an acrylic resin, a polyvinyl chloride resin, a polyvinylidene chloride resin, a polystyrene resin, a polyvinyl acetate resin, a styrene-butadiene copolymer, a vinylidene chloride-acrylonitrile copolymer, a vinyl chloride-vinyl acetate copolymer, a vinyl chloride-vinyl acetate-maleic anhydride copolymer, a silicone resin, a silicone alkyd resin, a phenol-formaldehyde resin, a styrene-alkyd resin, poly-N-vinylcarbazole, and polysilane. Among the above, for example, a polycarbonate resin or a polyarylate resin is preferable as the binder resin. The binder resins may be used alone or in combination of two or more kinds thereof.

A blending ratio between the charge transport material and the binder resin is, for example, preferably 10:1 to 1:5 in terms of mass ratio.

The charge transport layer may also contain other known additives.

The formation of the charge transport layer is not particularly limited, and a known forming method is used. For example, a coating film of a coating solution for forming the charge transport layer, in which the above-described components are added to a solvent, is formed, and the coating film is dried and then heated as necessary.

Examples of the solvent for preparing the coating solution for forming the charge transport layer include typical organic solvents, for example, aromatic hydrocarbons such as benzene, toluene, xylene, and chlorobenzene; ketones such as acetone and 2-butanone; halogenated aliphatic hydrocarbons such as methylene chloride, chloroform, and ethylene chloride; and cyclic or linear ethers such as tetrahydrofuran and ethyl ether. The solvents are used alone or in a form of a mixture of two or more kinds thereof.

Examples of the coating method of coating the charge generation layer with the coating solution for forming the charge transport layer include typical methods such as a blade coating method, a wire bar coating method, a spray coating method, a dip coating method, a bead coating method, an air knife coating method, and a curtain coating method.

A film thickness of the charge transport layer is set to, for example, preferably in a range of 5 µm or more and 50 µm or less and more preferably in a range of 10 µm or more and 30 µm or less.

### [Protective Layer]

A protective layer is provided on the charge transport layer as necessary. The protective layer is provided, for example, for the purpose of preventing a chemical change in the photosensitive layer during charging and further improving a mechanical strength of the photosensitive layer.

Here, a technique of forming an inorganic protective layer on the charge transport layer has been known in the related art. The charge transport layer tends to be flexible and easily deformable, while the inorganic protective layer tends to be hard but inferior in toughness. Therefore, the inorganic protective layer may be cracked.

For example, in a development step, in a case where a carrier is scattered from a developing unit and the scattered carrier is attached to the electrophotographic photoreceptor, the carrier reaches a transfer position while being attached to the electrophotographic photoreceptor. At the transfer position, a pressing force is applied in a state in which the carrier is interposed between the electrophotographic photoreceptor and a transferring unit. Therefore, in the inorganic protective layer, for example, cracking may occur due to friction of the carrier between the electrophotographic photoreceptor and the transferring unit.

In order to improve a mechanical strength of the inorganic protective layer, for example, it is considered to increase a thickness of the inorganic protective layer. However, in a case where the thickness of the inorganic protective layer is increased, charge is likely to be accumulated in the inorganic protective layer, and thus the residual potential may increase.

Here, the electrophotographic photoreceptor according to the present exemplary embodiment contains the metal oxide particles in the charge transport layer.

It is considered that the metal oxide particles function as a reinforcing material of the charge transport layer due to the filler effect. Therefore, it is considered that the charge transport layer is less likely to be deformed and the cracking of the inorganic protective layer is suppressed.

In addition, in the electrophotographic photoreceptor according to the present exemplary embodiment, as described above, the metal oxide particles are less likely to be aggregated in the charge transport layer and are dispersed in a state of having a small particle diameter and being close to uniform. As a result, the scattering of light in the charge transport layer can be suppressed, and the decrease in light transmittance can be suppressed.

### (Inorganic Protective Layer)

The inorganic protective layer is an inorganic material layer. Examples of the inorganic material include metal oxides such as gallium oxide, aluminum oxide, zinc oxide, titanium oxide, indium oxide, tin oxide, and boron oxide; metal nitrides such as gallium nitride, aluminum nitride, zinc nitride, titanium nitride, indium nitride, tin nitride, and boron nitride; carbon-based or silicon-based inorganic materials such as diamond-like carbon, amorphous carbon, hydrogenated amorphous carbon, hydrogenated and fluorinated amorphous carbon, amorphous silicon carbide, hydrogenated amorphous silicon carbide, amorphous silicon, and hydrogenated amorphous silicon; and mixed crystals thereof.

From the viewpoint of abrasion resistance and electrical properties of the photoreceptor, the inorganic protective layer is, for example, preferably a layer containing a metal oxide, more preferably a layer containing Group 13 element and an oxygen element, and still more preferably a layer containing gallium oxide or a layer containing aluminum oxide. The inorganic protective layer may contain one metal oxide or two or more metal oxides.

From the viewpoint of maintaining an electrostatic latent image, a volume resistivity of the inorganic protective layer is, for example, preferably 1.0 × 10¹⁰ Ω·cm or more, and more preferably 1.0 × 10¹¹ Ω·cm or more.

A method of measuring the volume resistivity of the inorganic protective layer is as follows.

The inorganic protective layer is peeled off from the photoreceptor and used as a sample. The sample is sandwiched in a sample holder of an impedance analyzer (Toyo Corporation), the resistance value is measured at an AC voltage of 1 V and a frequency of 100 Hz, and the calculation is performed based on the area of an electrode and the thickness of the sample.

Examples of a method of forming the inorganic protective layer include known vapor phase film forming methods such as plasma chemical vapor deposition (CVD), organic metal vapor phase growth, molecular beam epitaxy, vapor deposition, and sputtering. For example, the inorganic protective layer can be formed by applying the plasma CVD film deposition device and film deposition conditions described in JP2014-191179A.

From the viewpoint of abrasion resistance and electrical properties of the photoreceptor, a layer thickness of the inorganic protective layer is, for example, preferably 0.2 µm or more and 10 µm or less, more preferably 0.4 µm or more and 8 µm or less, and still more preferably 0.6 µm or more and 6 µm or less.

The film thickness of each layer of the photosensitive layer is an arithmetic average of measured values measured with an electromagnetic film thickness meter, and measurement points are four points in a circumferential direction at intervals of 90° in the center of the photoreceptor in the axial direction.

### [Image Forming Apparatus (and Process Cartridge)]

The image forming apparatus according to the present exemplary embodiment includes the electrophotographic photoreceptor, a charging device that charges a surface of the electrophotographic photoreceptor, an electrostatic latent image forming device that forms an electrostatic latent image on the charged surface of the electrophotographic photoreceptor, a developing device that develops the electrostatic latent image formed on the surface of the electrophotographic photoreceptor with a developer containing a toner to form a toner image, and a transfer device that transfers the toner image to a surface of a recording medium. The above-described electrophotographic photoreceptor according to the present exemplary embodiment is adopted as the electrophotographic photoreceptor.

As the image forming apparatus according to the present exemplary embodiment, a known image forming apparatus such as an apparatus including a fixing device that fixes the toner image transferred to the surface of a recording medium; a direct transfer-type apparatus that transfers the toner image formed on the surface of the electrophotographic photoreceptor directly to the recording medium; an intermediate transfer-type apparatus that primarily transfers the toner image formed on the surface of the electrophotographic photoreceptor to a surface of an intermediate transfer member and secondarily transfers the toner image transferred to the surface of the intermediate transfer member to the surface of the recording medium; an apparatus including a cleaning device that cleans the surface of the electrophotographic photoreceptor after the transfer of the toner image and before the charging; an apparatus including a charge erasing device that erases the charges on the surface of the electrophotographic photoreceptor by applying the charge erasing light after the transfer of the toner image and before the charging; or an apparatus including an electrophotographic photoreceptor heating member for increasing the temperature of the electrophotographic photoreceptor and decreasing the relative temperature is adopted.

In a case of the intermediate transfer-type apparatus, the transfer device has a configuration including an intermediate transfer member with surface on which the toner image will be transferred, a primary transfer device that performs primary transfer to transfer the toner image formed on the surface of the electrophotographic photoreceptor to the surface of the intermediate transfer member, and a secondary transfer device that performs secondary transfer to transfer the toner image transferred to the surface of the intermediate transfer member to the surface of a recording medium.

The image forming apparatus according to the present exemplary embodiment may be any of a dry development-type image forming apparatus or a wet development-type (development type using a liquid developer) image forming apparatus.

In the image forming apparatus according to the present exemplary embodiment, for example, a portion including the electrophotographic photoreceptor may have a cartridge structure (process cartridge) that is attachable to and detachable from the image forming apparatus. As the process cartridge, for example, a process cartridge including the electrophotographic photoreceptor according to the present exemplary embodiment is preferably used. The process cartridge may include, for example, at least one selected from the group consisting of a charging device, an electrostatic latent image forming device, a developing device, and a transfer device, in addition to the electrophotographic photoreceptor.

An example of the image forming apparatus according to the present exemplary embodiment will be shown below, but the present invention is not limited thereto. Hereinafter, among the parts shown in the drawing, main parts will be described, and others will not be described.

Fig. 2 is a view schematically showing a configuration of an example of the image forming apparatus according to the present exemplary embodiment.

As shown in Fig. 2, an image forming apparatus 100 according to the present exemplary embodiment includes a process cartridge 300 including an electrophotographic photoreceptor 7, an exposure device 9 (an example of the electrostatic latent image forming device), a transfer device 40 (primary transfer device), and an intermediate transfer member 50. In the image forming apparatus 100, the exposure device 9 is disposed at a position that can be exposed to the electrophotographic photoreceptor 7 from an opening portion of the process cartridge 300; the transfer device 40 is disposed at a position that faces the electrophotographic photoreceptor 7 through the intermediate transfer member 50; and the intermediate transfer member 50 is disposed such that a part of the intermediate transfer member 50 is in contact with the electrophotographic photoreceptor 7. Although not shown, the image forming apparatus also includes a secondary transfer device that transfers the toner image transferred to the intermediate transfer member 50 to a recording medium (for example, paper). The intermediate transfer member 50, the transfer device 40 (primary transfer device), and the secondary transfer device (not shown) correspond to an example of the transfer device.

The process cartridge 300 in Fig. 2 integrally supports the electrophotographic photoreceptor 7, a charging device 8 (an example of the charging device), a developing device 11 (an example of the developing device), and a cleaning device 13 (an example of the cleaning device) in a housing. The cleaning device 13 has a cleaning blade (an example of a cleaning member) 131, and the cleaning blade 131 is disposed to come into contact with the surface of the electrophotographic photoreceptor 7. The cleaning member may be a conductive or insulating fibrous member instead of the aspect of the cleaning blade 131, and may be used alone or in combination with the cleaning blade 131.

Fig. 2 shows an example of an image forming apparatus including a fibrous member 132 (roll shape) that supplies a lubricant 14 to the surface of the electrophotographic photoreceptor 7 and a fibrous member 133 (flat brush shape) that assists the cleaning, but these are disposed as necessary.

Hereinafter, each configuration of the image forming apparatus according to the present exemplary embodiment will be described.

### -Charging Device-

As the charging device 8, for example, a contact-type charger formed of a conductive or semi-conductive charging roller, a charging brush, a charging film, a charging rubber blade, a charging tube, or the like is used. In addition, a known charger such as a non-contact type roller charger, and a scorotoron charger or a corotron charger using corona discharge is also used.

### -Exposure Device-

Examples of the exposure device 9 include an optical system device that exposes the surface of the electrophotographic photoreceptor 7 to light such as a semiconductor laser beam, LED light, and liquid crystal shutter light in a predetermined image pattern. A wavelength of the light source is within the spectral sensitivity region of the electrophotographic photoreceptor. As a wavelength of a semiconductor laser, near infrared laser, which has an oscillation wavelength in the vicinity of 780 nm, is mostly used. However, the wavelength is not limited thereto, and a laser having an oscillation wavelength of an approximately 600 nm level or a laser having an oscillation wavelength of 400 nm or more and 450 nm or less as a blue laser may also be used. In addition, a surface emission-type laser light source capable of outputting a multibeam is also effective for forming a color image.

### -Developing Device-

Examples of the developing device 11 include a typical developing device that performs development in contact or non-contact with the developer. The developing device 11 is not particularly limited as long as the device has the above-described functions, and is selected depending on the purpose thereof. Examples thereof include known developing machines having a function of attaching a one-component developer or a two-component developer to the electrophotographic photoreceptor 7 using a brush, a roller, or the like. Among the above, for example, a developing roller in which a developer is retained on a surface is preferably used.

The developer used in the developing device 11 may be a one-component developer containing only a toner or a two-component developer containing a toner and a carrier. In addition, the developer may be magnetic or non-magnetic. Known developers are employed as the developer.

### -Cleaning Device-

As the cleaning device 13, a cleaning blade-type device including the cleaning blade 131 is used.

In addition to the cleaning blade-type device, a fur brush cleaning-type device or a simultaneous development cleaning-type device may be adopted.

### -Transfer Device-

Examples of the transfer device 40 include a known transfer charger such as a contact type transfer charger using a belt, a roller, a film, a rubber blade, or the like, and a scorotron transfer charger or a corotron transfer charger using corona discharge.

### -Intermediate Transfer Member-

As the intermediate transfer member 50, a semi-conductive belt-like intermediate transfer member (intermediate transfer belt) containing polyimide, polyamide-imide, polycarbonate, polyarylate, polyester, rubber, or the like is used. In addition, as the form of the intermediate transfer member, a drum-like intermediate transfer member may be used in addition to the belt-like intermediate transfer member.

Fig. 3 is a view schematically showing a configuration of another example of the image forming apparatus according to the present exemplary embodiment.

An image forming apparatus 120 shown in Fig. 3 is a tandem type multicolor image forming apparatus in which four process cartridges 300 are mounted. The image forming apparatus 120 is formed such that the four process cartridges 300 are arranged in parallel on the intermediate transfer member 50, and one electrophotographic photoreceptor is used for each color. The image forming apparatus 120 has the same configuration as the image forming apparatus 100, except that the image forming apparatus 120 is of a tandem type.

### Examples

Hereinafter, exemplary embodiments of the invention will be specifically described based on examples. However, the exemplary embodiments of the invention are not limited to the examples.

In the following description, unless otherwise specified, "parts" and "%" are based on mass.

In the following description, the synthesis, the production, the treatment, the measurement, and the like are carried out at normal temperature (25°C ± 3°C), unless otherwise specified.

### <Example 1>

### [Formation of Undercoat Layer]

An aluminum cylindrical tube having an outer diameter of 30 mm, a length of 250 mm, and a thickness of 1 mm is prepared as a conductive substrate.

100 parts of zinc oxide (average particle size: 70 nm, specific surface area: 15 m²/g, Tayca Corporation) is stirred and mixed with 500 parts of toluene, 1.3 parts of a silane coupling agent (trade name: KBM603, Shin-Etsu Chemical Co., Ltd., N-2-(aminoethyl)-3-aminopropyltrimethoxysilane) is added thereto, and the mixture is stirred for 2 hours. Next, the toluene is distilled off under reduced pressure and baked at 120°C for 3 hours to obtain zinc oxide subjected to a surface treatment with the silane coupling agent.

110 parts of the surface-treated zinc oxide is stirred and mixed with 500 parts of tetrahydrofuran, a solution obtained by dissolving 0.6 parts of alizarin in 50 parts of tetrahydrofuran is added thereto, and the mixture is stirred at 50°C for 5 hours. Next, the solid content is separated by filtration by carrying out filtration under reduced pressure, and dried at 60°C under reduced pressure, thereby obtaining zinc oxide with alizarin.

100 parts of a solution obtained by dissolving 60 parts of the zinc oxide with alizarin, 13.5 parts of a curing agent (blocked isocyanate, trade name: SUMIDUR 3175, Sumitomo Bayer Urethane Co., Ltd.), and 15 parts of a butyral resin (trade name: S-LEC BM-1, Sekisui Chemical Co., Ltd.) in 68 parts of methyl ethyl ketone is mixed with 5 parts of methyl ethyl ketone, and the mixture is dispersed in a sand mill for 2 hours using glass beads with a diameter of 1 mm, thereby obtaining a dispersion. 0.005 parts of dioctyl tin dilaurate as a catalyst and 4 parts of silicone resin particles (trade name: TOSPEARL 145, Momentive Performance Materials Inc.) are added to the dispersion to obtain a coating solution for forming an undercoat layer. The outer peripheral surface of the conductive substrate is coated with the coating solution for forming an undercoat layer by dip coating, and dried and cured at 170°C for 40 minutes to form an undercoat layer with a layer thickness of 20 µm.

### [Formation of Charge Generation Layer]

A mixture of 15 parts of hydroxygallium phthalocyanine as a charge generation material (having diffraction peaks at positions where Bragg angles (2θ ± 0.2°) in the X-ray diffraction spectrum using CuKα characteristic X-rays are at least of 7.5°, 9.9°, 12.5, 16.3°, 18.6°, 25.1°, and 28.3°), 10 parts of a vinyl chloride-vinyl acetate copolymer resin (trade name: VMCH, manufactured by Nippon Unicar Company Limited) as a binder resin, and 200 parts of n-butyl acetate is dispersed in a sand mill for 4 hours using glass beads with a diameter of 1 mm. 175 parts of n-butyl acetate and 180 parts of methyl ethyl ketone are added to the dispersion, and the mixture is stirred to obtain a coating solution for forming a charge generation layer. The undercoat layer is dipped in and coated with the coating solution for forming a charge generation layer, and dried at normal temperature to form a charge generation layer having a layer thickness of 0.25 µm.

### [Formation of Charge Transport Layer]

· Binder resin: polycarbonate resin (1) (viscosity-average molecular weight: 40,000, numerical values in structural formulae indicate molar ratios) ... 20 parts
· Charge transport material: CTM-1 ... 15 parts
· Metal oxide particles: silica particles hydrophobized with 1,1,1,3,3,3-hexamethyldisilazane (average particle diameter: 150 nm, average circularity: 0.85, degree of hydrophobicity: 65%) ... amount such that volume (% ) shown in Table 1 is obtained
· Solvent: tetrahydrofuran (THF) ... 600 parts

The above-described materials are stirred and mixed for 12 hours to obtain a coating solution for forming a charge transport layer. The charge generation layer is coated with the coating solution for forming a charge transport layer by dip coating under a condition of a room temperature of 28°C. Thereafter, hot air is blown to the coating film to dry the coating film, thereby forming a charge transport layer having a layer thickness of 30 µm.

A photoreceptor is obtained through the above-described steps.

### <Example 2>

A photoreceptor is obtained in the same manner as in Example 1, except that the charge transport layer is formed by dip coating under a condition of room temperature of 30°C.

### <Example 3>

A photoreceptor is obtained in the same manner as in Example 1, except that the charge transport layer is formed by dip coating under a condition of room temperature of 32°C.

### <Example 4>

A photoreceptor is obtained in the same manner as in Example 1, except that, in the formation of the charge transport layer, the addition amount of the silica particles is changed as shown in Table 1, and the stirring and mixing time of the materials is set to 6 hours.

### <Example 5>

A photoreceptor is obtained in the same manner as in Example 1, except that, in the formation of the charge transport layer, the addition amount of the silica particles is changed as shown in Table 1, and the stirring and mixing time of the materials is set to 8 hours.

### <Example 6>

A photoreceptor is obtained in the same manner as in Example 1, except that, in the formation of the charge transport layer, the addition amount of the silica particles is changed as shown in Table 1, and the stirring and mixing time of the materials is set to 14 hours.

### <Example 7>

A photoreceptor is obtained in the same manner as in Example 1, except that, in the formation of the charge transport layer, the addition amount of the silica particles is changed as shown in Table 1, and the stirring and mixing time of the materials is set to 16 hours.

### <Example 8>

A photoreceptor is obtained in the same manner as in Example 1, except that, in the formation of the charge transport layer, the silica particles are changed to zinc oxide particles having an average circularity of 0.6 and a degree of hydrophobicity of 65%.

### <Example 9>

A photoreceptor is obtained in the same manner as in Example 1, except that, in the formation of the charge transport layer, the average circularity of the silica particles is changed to 0.6.

### <Example 10>

A photoreceptor is obtained in the same manner as in Example 1, except that, in the formation of the charge transport layer, the average circularity of the silica particles is changed to 0.7.

### <Example 11>

A photoreceptor is obtained in the same manner as in Example 1, except that, in the formation of the charge transport layer, the average circularity of the silica particles is changed to 0.8.

### <Example 12>

A photoreceptor is obtained in the same manner as in Example 1, except that, in the formation of the charge transport layer, the degree of hydrophobicity of the silica particles is changed to 55%.

### <Example 13>

A photoreceptor is obtained in the same manner as in Example 1, except that, in the formation of the charge transport layer, 200 parts in the solvent of 600 parts of THF are changed to 200 parts of toluene.

### <Example 14>

A photoreceptor is obtained in the same manner as in Example 1, except that, in the formation of the charge transport layer, 100 parts in the solvent of 600 parts of THF are changed to 100 parts of toluene.

### <Example 15>

A photoreceptor is obtained in the same manner as in Example 1, except that an inorganic protective layer is formed on the charge transport layer as follows.

### -Formation of Inorganic Protective Layer-

An amorphous layer containing gallium oxide is formed as an inorganic protective layer by plasma CVD using trimethylgallium as a film forming material. A layer thickness thereof is 3 µm.

### <Comparative Example 1>

Each photoreceptor is produced by changing the room temperature during the dip coating to 22°C from Example 1.

### <Various Measurements>

The following items are measured by the methods described above.
· Proportion (% by number) of the single particles of the metal oxide particles contained in the charge transport layer: indicated by "A1/(A1 + A2)" in Table 1
· Proportion (%) of the total area of the single particles and the aggregated particles of the metal oxide particles contained in the charge transport layer
· Average circularity and degree of hydrophobicity of the metal oxide particles

### <Performance Evaluation of Photoreceptor>

### [Hardness]

A hardness of the charge transport layer of each example is evaluated as follows.

A hardness of an outer peripheral surface of the photoreceptor is a Young's modulus (GPa) obtained by a nanoindentation method. The axial direction of the photoreceptor is fixed to the horizontal direction, and the hardness is measured at the apex in the center of the axial direction of the photoreceptor.

Young's moduli at four positions are measured at intervals of 90° in the circumferential direction of the photoreceptor, and the Young's moduli at the four positions are arithmetically averaged.

Measurement conditions with the nanoindenter are as follows.

The measurement results are shown in Table 1.
· Test device: product name PICODENTOR^{®} HM-500, Fisher Instruments K.K.
· Indenter: diamond triangular indenter with an angle of 115°
· Load: 75 mN

### [Abrasion Resistance]

Abrasion resistance of the photoreceptor of each example is evaluated as follows.

The photoreceptor of each example is mounted on an electrophotographic image forming apparatus (manufactured by FUJIFII,M Business Innovation Corp., Apeos C4570), and 100,000 sheets of A3-sized paper are formed with a 1% solid image and an image with an image density (area coverage) of 1% in an environment of a temperature of 30°C and a relative humidity of 85%. Thereafter, a 100% solid image as a solid image with an image density (area coverage) of 100% is formed on 100,000 sheets of A3 size paper in an environment of a temperature of 10°C and a relative humidity of 15%. The above-described image formation (that is, the formation of 200,000 images in total of the formation of 100,000 images in the environment of a temperature of 30°C and a relative humidity of 85% and the formation of 100,000 images in the environment of a temperature of 10°C and a relative humidity of 15%) is repeated 5 times. The average thickness of the charge transport layer is obtained before and after the above-described image formation (that is, the formation of the total of 1,000,000 images), and the difference in average thickness before and after the image formation is defined as an abrasion amount (nm). PERMASCOPE manufactured by Fisher Instruments K.K. is used as a film thickness measuring machine.

The abrasion amount is classified as follows. The results are shown in Table 1.
G1: abrasion amount is less than 500 nm.
G2: abrasion amount is 500 nm or more and less than 1,000 nm.
G3: abrasion amount is 1,000 nm or more and less than 1,500 nm.
G4: abrasion amount is 1,500 nm or more.

### [Electrical Properties]

Electrical properties of the charge transport layer of each example are evaluated as follows.

In an environment of a temperature of 22°C and a relative humidity of 55%, the photoreceptor is rotated at a rotation speed of 40 rpm, and while the surface of the photoreceptor is scanned, the surface of the photoreceptor is irradiated with light for exposure (light source: semiconductor laser, wavelength: 780 nm, output: 5 mW) in a state of being negatively charged to -700 V by a scorotoron charger. Thereafter, a residual potential of the surface of the photosensitive body is measured.

For the potential measurement, a surface potential probe of a surface potential meter (manufactured by TREK INC., TREK 334), that is installed at a position at the center of the photoreceptor in the axial direction and 1 mm away from the surface of the photoreceptor, is used.

The measured residual potential is classified into the following G1 to G4, and the effect of suppressing an increase in residual potential is evaluated. A voltage of less than 40 V is determined to be acceptable. The results are shown in Table 1.
G1: less than 15 V
G2: 15 V or more and less than 30 V
G3: 30 V or more and less than 40 V
G4: 40 V or more

### [Cracking Resistance of Inorganic Protective Layer]

A cracking load of the inorganic protective layer is measured as follows to evaluate cracking resistance of the inorganic protective layer.

Measurement by a hardness test using a microhardness tester is repeated while increasing the load from 0 mN to 5 mN. By observation with an optical microscope each time the load is applied, a load at which the inorganic protective layer is cracked is defined as a cracking initiation load. The measurement conditions are as follows.
· Test device: product name DUH-201, Shimadzu Corporation
· Indenter: diamond spherical indenter

**[Table 1]**

| | Charge transport layer | | | | | | | | | Inorganic protective layer | Evaluation | | | |
|---|---|---|---|---|---|---|---|---|---|---|---|---|---|---|
| | Metal oxide particles | | | | | | | | Light transmittance % | | Hardness GPa | Abrasion resistance | Electrical properties | Cracking resistance of inorganic protective layer |
| | Type of metal oxide | Number of single particles A1 | Number of aggregated particles A2 | % by number of A1/(A1 + A2) | Proportion % of total area of single particles and aggregated particles | Volume ratio % of metal oxide particles (material) added amount) | Average circularity | Degree of hydrophobicity % | | Presence or absence | | | | |
| Example 1 | Silica particles | 60 | 40 | 60 | 80 | 60 | 0.85 | 65 | 90 | N | 10 | G1 | G3 | - |
| Example 2 | Silica particles | 70 | 30 | 70 | 80 | 60 | 0.85 | 65 | 90 | N | 13 | G1 | G2 | - |
| Example 3 | Silica particles | 90 | 10 | 90 | 80 | 60 | 0.85 | 65 | 90 | N | 15 | G1 | G1 | - |
| Example 4 | Silica particles | 60 | 40 | 60 | 55 | 45 | 0.85 | 65 | 90 | N | 10 | G3 | G1 | - |
| Example 5 | Silica particles | 60 | 40 | 60 | 60 | 50 | 0.85 | 65 | 90 | N | 11 | G2 | G1 | - |
| Example 6 | Silica particles | 60 | 40 | 60 | 95 | 65 | 0.85 | 65 | 90 | N | 14 | G1 | G2 | - |
| Example 7 | Silica particles | 60 | 40 | 60 | 98 | 66 | 0.85 | 65 | 90 | N | 15 | G1 | G3 | - |
| Example 8 | Zinc oxide particles | 60 | 40 | 60 | 80 | 60 | 0.85 | 65 | 90 | N | 8 | G1 | G1 | - |
| Example 9 | Silica particles | 60 | 40 | 60 | 80 | 60 | 0.6 | 65 | 90 | N | 8 | G1 | G1 | - |
| Example 10 | Silica particle | 60 | 40 | 60 | 80 | 60 | 0.7 | 65 | 90 | N | 9 | G1 | G1 | - |
| Example 11 | Silica particle | 60 | 40 | 60 | 80 | 60 | 0.8 | 65 | 90 | N | 10 | G1 | G1 | - |
| Example 12 | Silica particle | 60 | 40 | 60 | 80 | 60 | 0.85 | 55 | 90 | N | 10 | G1 | G3 | - |
| Example 13 | Silica particle | 60 | 40 | 60 | 80 | 60 | 0.85 | 65 | 75 | N | 10 | G1 | G3 | - |
| Example 14 | Silica particle | 60 | 40 | 60 | 80 | 60 | 0.85 | 65 | 80 | N | 10 | G1 | G2 | - |
| Example 15 | Silica particle | 60 | 40 | 60 | 80 | 60 | 0.85 | 65 | 90 | Y | - | G1 | G1 | 100 |
| Comparative Example 1 | Silica particles | 60 | 40 | 50 | 80 | 60 | 0.85 | 65 | 90 | N | 10 | G1 | G4 | - |

From the above results, it is found that the photoreceptors of Examples have both abrasion resistance and electrical properties higher than those of the photoreceptor of Comparative Example.

The present exemplary embodiments include the following aspects.
(((1))) An electrophotographic photoreceptor comprising:
   a conductive substrate;
   a charge generation layer that is disposed on the conductive substrate; and
   a charge transport layer that is disposed on the charge generation layer and contains a binder resin, a charge transport material, and metal oxide particles,
   wherein, in a case where a cross section of the charge transport layer is observed, a proportion of single particles of the metal oxide particles to a total of the single particles and aggregated particles of the metal oxide particles is 60% by number or more.
(((2))) The electrophotographic photoreceptor according to (((1))),
   wherein the proportion of the single particles of the metal oxide particles is 70% by number or more.
(((3))) The electrophotographic photoreceptor according to (((1))) or (((2))),
   wherein, in the case where the cross section of the charge transport layer is observed, a proportion of a total area of the single particles and the aggregated particles of the metal oxide particles to an area of an entire observed cross section is 60% by area or more and 95% by area or less.
(((4))) The electrophotographic photoreceptor according to any one of (((1))) to (((3))),
   wherein the metal oxide particles are silica particles.
(((5))) The electrophotographic photoreceptor according to any one of (((1))) to (((4))),
   wherein, in the metal oxide particles, an average circularity is 0.7 or more and a degree of hydrophobicity is 60% or more.
(((6))) The electrophotographic photoreceptor according to (((5))),
   wherein, in the metal oxide particles, the average circularity is 0.8 or more and the degree of hydrophobicity is 60% or more.
(((7))) The electrophotographic photoreceptor according to any one of (((1))) to (((6))),
   wherein a light transmittance T of the charge transport layer is 80% or more.
(((8))) The electrophotographic photoreceptor according to any one of (((1))) to (((7))), further comprising:
   an inorganic protective layer that is disposed on the charge transport layer.
(((9))) A process cartridge comprising:
   the electrophotographic photoreceptor according to any one of (((1))) to (((8))),
   wherein the process cartridge is attachable to and detachable from an image forming apparatus.
(((10))) An image forming apparatus comprising:
   the electrophotographic photoreceptor according to any one of (((1))) to (((8)));
   a charging device that charges a surface of the electrophotographic photoreceptor;
   an electrostatic latent image forming device that forms an electrostatic latent image on the charged surface of the electrophotographic photoreceptor;
   a developing device that develops the electrostatic latent image formed on the surface of the electrophotographic photoreceptor with a developer containing a toner to form a toner image; and
   a transfer device that transfers the toner image to a surface of a recording medium.

The effects of the above-described aspects are as follows.

According to (((1))), there is provided an electrophotographic photoreceptor including a conductive substrate, a charge generation layer that is disposed on the conductive substrate, and a charge transport layer that is disposed on the charge generation layer and contains a binder resin, a charge transport material, and metal oxide particles, in which the electrophotographic photoreceptor has excellent abrasion resistance and electrical properties, as compared with a case where, when a cross section of the charge transport layer is observed, a proportion of single particles of the metal oxide particles to a total of the single particles and aggregated particles of the metal oxide particles is less than 60% by number.

According to (((2))), there is provided an electrophotographic photoreceptor having excellent abrasion resistance and electrical properties, as compared with a case where the proportion of the single particles of the metal oxide particles is less than 70% by number.

According to (((3))), there is provided an electrophotographic photoreceptor having excellent abrasion resistance and electrical properties, as compared with a case where, when the cross section of the charge transport layer is observed, a proportion of a total area of the single particles and the aggregated particles of the metal oxide particles to an area of an entire observed cross section is less than 60% by area or more than 95% by area.

According to (((4))), there is provided an electrophotographic photoreceptor having excellent abrasion resistance and electrical properties, as compared with a case where the metal oxide particles are not silica particles.

According to (((5))) or (((6))), there is provided an electrophotographic photoreceptor having excellent abrasion resistance and electrical properties, as compared with a case where the average circularity of the metal oxide particles is less than 0.7 or the degree of hydrophobicity thereof is less than 60%, or a case where the average circularity of the metal oxide particles is less than 0.8 or the degree of hydrophobicity thereof is less than 60%.

According to (((7))), there is provided an electrophotographic photoreceptor having excellent abrasion resistance and electrical properties, as compared with a case where the light transmittance T of the charge transport layer is less than 80%.

According to (((8))), there is provided an electrophotographic photoreceptor including a conductive substrate, a charge generation layer that is disposed on the conductive substrate, and a charge transport layer that is disposed on the charge generation layer and contains a binder resin, a charge transport material, and metal oxide particles, in which the electrophotographic photoreceptor has excellent cracking prevention in an inorganic protective layer and electrical properties, as compared with a case where, when a cross section of the charge transport layer is observed, a proportion of single particles of the metal oxide particles to a total of the single particles and aggregated particles of the metal oxide particles is less than 60% by number.

According to (((9))) or (((10))), there is provided a process cartridge or an image forming apparatus, each of which includes an electrophotographic photoreceptor including a conductive substrate, a charge generation layer that is disposed on the conductive substrate, and a charge transport layer that is disposed on the charge generation layer and contains a binder resin, a charge transport material, and metal oxide particles, in which the electrophotographic photoreceptor has excellent abrasion resistance and electrical properties, as compared with a case of adopting an electrophotographic photoreceptor in which, in a case where a cross section of the charge transport layer is observed, a proportion of single particles of the metal oxide particles to a total of the single particles and aggregated particles of the metal oxide particles is less than 60% by number.

The foregoing description of the exemplary embodiments of the present invention has been provided for the purposes of illustration and description. It is not intended to be exhaustive or to limit the invention to the precise forms disclosed. Obviously, many modifications and variations will be apparent to practitioners skilled in the art. The embodiments were chosen and described in order to best explain the principles of the invention and its practical applications, thereby enabling others skilled in the art to understand the invention for various embodiments and with the various modifications as are suited to the particular use contemplated. It is intended that the scope of the invention be defined by the following claims and their equivalents.

### Brief Description of the Reference Symbols

1: conductive substrate
2: undercoat layer
3: charge generation layer
4: charge transport layer
5: photosensitive layer
6: inorganic protective layer
10A: photoreceptor
7: electrophotographic photoreceptor
8: charging device
9: exposure device
11: developing device
13: cleaning device
14: lubricant
40: transfer device
50: intermediate transfer member
100: image forming apparatus
120: image forming apparatus
131: cleaning blade
132: fibrous member (roll shape)
133: fibrous member (flat brush shape)
300: process cartridge

## Claims

1. An electrophotographic photoreceptor comprising:
a conductive substrate;
a charge generation layer that is disposed on the conductive substrate; and
a charge transport layer that is disposed on the charge generation layer and contains a binder resin, a charge transport material, and metal oxide particles,
wherein, in a case where a cross section of the charge transport layer is observed, a proportion of single particles of the metal oxide particles to a total of the single particles and aggregated particles of the metal oxide particles is 60% by number or more.

2. The electrophotographic photoreceptor according to claim 1,
wherein the proportion of the single particles of the metal oxide particles is 70% by number or more.

3. The electrophotographic photoreceptor according to claim 1 or 2,
wherein, in the case where the cross section of the charge transport layer is observed, a proportion of a total area of the single particles and the aggregated particles of the metal oxide particles to an area of an entire observed cross section is 60% by area or more and 95% by area or less.

4. The electrophotographic photoreceptor according to any one of claims 1 to 3,
wherein the metal oxide particles are silica particles.

5. The electrophotographic photoreceptor according to any one of claims 1 to 4,
wherein, in the metal oxide particles, an average circularity is 0.7 or more and a degree of hydrophobicity is 60% or more.

6. The electrophotographic photoreceptor according to claim 5,
wherein, in the metal oxide particles, the average circularity is 0.8 or more and the degree of hydrophobicity is 60% or more.

7. The electrophotographic photoreceptor according to any one of claims 1 to 6,
wherein a light transmittance T of the charge transport layer is 80% or more.

8. The electrophotographic photoreceptor according to any one of claims 1 to 7, further comprising:
an inorganic protective layer that is disposed on the charge transport layer.

9. A process cartridge comprising:
the electrophotographic photoreceptor according to any one of claims 1 to 8,
wherein the process cartridge is attachable to and detachable from an image forming apparatus.

10. An image forming apparatus comprising:
the electrophotographic photoreceptor according to any one of claims 1 to 8;
a charging device that charges a surface of the electrophotographic photoreceptor;
an electrostatic latent image forming device that forms an electrostatic latent image on the charged surface of the electrophotographic photoreceptor;
a developing device that develops the electrostatic latent image formed on the surface of the electrophotographic photoreceptor with a developer containing a toner to form a toner image; and
a transfer device that transfers the toner image to a surface of a recording medium.
